

Oct. 19, 1965

B. ASNES

3,212,924

NON-CURLING GUMMED PAPER AND METHOD OF MAKING

Filed July 6, 1962



INVENTOR.

*Benjamin Asnes*  
BY  
*Roberts, Cahnman & Grover*  
ATT'YS

## 1

3,212,924

### NON-CURLING GUMMED PAPER AND METHOD OF MAKING

Benjamin Asnes, Framingham, Mass., assignor to Dennison Manufacturing Company, a corporation of Nevada

Filed July 6, 1962, Ser. No. 208,076  
10 Claims. (Cl. 117—122)

This is in part a continuation of Serial No. 692,253, filed October 25, 1957, and now abandoned.

This invention relates to gummed sheet material, that is, sheet material having a coating of dry adhesive which can be moistened with water to develop an adhesive tackiness which permits the sheet to be attached to another surface. Such coated sheets are common articles of commerce, gummed labels and postage stamps being common examples. Adhesives of this nature are commonly called "remoistenable" adhesives, glue or gum and these terms are herein used to include any normally non-tacky adhesive which can be activated with water.

Gummed sheet materials of this character have been troublesome in use because of their tendency to curl or roll up with changes in relative humidity due to the uneven expansion and contraction of the adhesive coating and of the backing sheet. This problem is particularly troublesome in gummed sheets which receive printing for labels and the like which have to be run through printing presses in controlled registration therewith. This difficulty has necessitated printing rooms with controlled relative humidity.

A number of expedients have heretofore been attempted to correct this problem but with only partial success. The most usual expedient adopted has been to break up the coated adhesive into small sections by drawing the coated sheet under tension over variously disposed edges. This method is only partially effective and requires an additional and troublesome operation. Another expedient used has been the inclusion of resilient fillers to minimize the differential effect of the expansion and contraction. This method is also only partially effective and increases the cost.

A recent expedient is disclosed in United States Patent No. 2,793,966. This method involves the dispersion of minute particles of solid water-reactivatable adhesive in a solvent solution of a second gum which is also water soluble. The solvent used for the dispersion dissolves the second or carrier gum which is present in a minor proportion when compared with the water-reactivatable adhesive, but in which the latter is not soluble. After coating and drying, the minute solid particles of water-reactivatable adhesive are presumably discontinuous in a matrix of the second gum. This method produces a gummed sheet of superior flatness but introduces its own problems. An important problem with this method is the necessity for obtaining the water-reactivatable adhesive in a very fine particle size, usually less than one mil. Such materials, being adhesive and moisture-sensitive, are extremely difficult to grind and maintain in this small particle size. Also this method requires substantial amounts of the second or carrier gum which is quite expensive when compared with the usual water-sensitive adhesive.

The principal object of this invention is to provide superflat gummed sheet material, together with a method

## 2

and coating composition for making the same which will remain substantially flat even after repeated changes in relative humidity. Further objects are to provide superflat gummed sheet material having an adhesive layer which is firmly bound to the carrier sheet, which will not block or adhere to superposed sheets when stacked with other sheets of like material, which is readily activated with water, which is easily prepared, and which is relatively inexpensive when compared with previous methods.

In accordance with this invention the improved superflat gummed sheet material of the water-remoistenable type comprises a sheet having on one side thereof a potentially adhesive dry film which when moistened with water will adhere to a surface, said film comprising in discontinuous phase a multiplicity of minute particles of water-soluble gum and in continuous phase of a resinous film-forming binder joining said particles together and to the sheet, said binder being substantially insoluble in water but sufficiently open to permit quick activation of said particles by water. The particles of water-soluble gum should comprise a major portion of the total mass of the film and the ratio of gum to binder should be at least about 4 to 1 by weight. Suitable binder materials are substantially water-insoluble polyvinyl ester copolymer, polyvinyl chloride, butadiene-styrene copolymers, and polymers of acrylic esters. The preferred and substantially superior binder is water-insoluble polyvinyl acetate copolymerized with a small proportion of material of the crotonic or maleic type. While the water-soluble gum is in discontinuous phase, the particles do adhere to each other to a slight extent and those in the inner stratum of the coating adhere directly to the carrier sheet. Indeed if the continuous phase is dissolved from the coating, the gum remains as a self-supporting porous structure. Likewise if the gum is extracted from the film, the resinous binder remains as an open, sponge-like structure.

The above superflat gummed sheet material is made by a method which comprises dissolving a substantially water-insoluble binder in a solvent or mixture of solvents which is incompletely miscible with water, dissolving a water-reactivatable gum in water, dispersing the water solution in the binder solution, coating the resulting composition on the sheet, and drying. After the coating has been dried the exposed surface of the carrier sheet should be treated under tension, according to techniques well known in the prior art, to equalize the contraction caused by wetting the coated side.

In a further aspect the present invention includes a 50 coatable composition for preparing water-remoistenable gummed sheet material comprising a dispersion of a water solution of water-reactivatable gum dispersed in a solution of substantially water-insoluble, resinous, film-forming binder in a solvent incompletely miscible with water, said gum exceeding by weight the amount of the binder.

To the naked eye the coatings of the present invention appear smooth and substantially homogeneous. However, microphotographs show rather clearly that the coatings, after drying, have particles of water-reactivatable adhesive embedded in a water-insoluble binder matrix. These particles are available to water as is illustrated by the ease with which the film is made tacky by moistening and by the fact that micro-photographs of samples

taken after prolonged immersion in water show that most of the gum particles are leached out by the water. The use of water-insoluble binder thus does not prevent the reactivation of the gum while providing resistance against the washing away of the coating and permitting the use of thinner coatings.

This invention can be illustrated by the following examples where all parts are parts by weight.

#### EXAMPLE I

##### (A)

Dissolve polyvinyl acetate copolymerized with a small proportion of material of the crotonic or maleic type ( $C_3V_{10}$  of the Shawinigan Products Corp.) in:

|                                                                                       |     |
|---------------------------------------------------------------------------------------|-----|
| Toluol                                                                                | 150 |
| Isopropanol                                                                           | 50  |
| Ethyl acetate                                                                         |     |
| Santicizer E15 (phthalate ethyl glycolate a plasticizer of the Monsanto Chemical Co.) | 10  |
| 17% ammonia solution                                                                  | 8   |

after a clear solution is obtained add:

and stir well.

##### (B)

|           |     |
|-----------|-----|
| Bone glue | 125 |
| Dextrin   | 65  |
| Water     | 210 |

Add ammonia (28%) to the water solution of the gum base (B) until it is slightly alkaline then add A slowly to A while stirring vigorously and then thin to a good coating viscosity by adding 20 to 30 parts of ethyl acetate to the dispersion.

Further examples illustrating a variety of water-insoluble resins which can be used are shown by the following:

| Example No.         | 2   | 3   | 4   | 5  | 6  |
|---------------------|-----|-----|-----|----|----|
| $C_3V_{10}$ resin   | 10  |     |     |    |    |
| Pliolite Latex #170 |     | 30  |     |    |    |
| Geon 200 x 20       |     |     | 10  |    |    |
| Acryloid B66        |     | 25  |     |    |    |
| Alvex (4cc-417)     | 6   |     |     | 20 |    |
| Toluol              | 60  | 80  | 35  | 50 |    |
| Acetone             | 10  |     |     | 15 |    |
| Ethyl Acetate       |     |     |     | 60 |    |
| Isopropanol         | 10  |     |     |    |    |
| Santicizer E15      | 4   |     | 4   |    | 4  |
| Diethyl phthalate   |     |     | 4   |    |    |
| Ammonia (17%)       | 3.2 | 3.2 | 3.2 |    |    |
| Animal glue         | 15  | 15  | 15  | 15 | 39 |
| Dextrin             | 25  | 25  | 25  | 25 | 21 |
| Water               | 40  | 40  | 40  | 40 | 60 |

"Pliolite Latex #170" is a 30% emulsion of a butadiene-styrene polymer of the Goodyear Tire & Rubber Co.

"Geon 200 x 20" is a polyvinyl chloride resin of the B. F. Goodrich Co.

"Acryloid B66" is a 40% solids in toluol of an acrylate of the Rohm & Haas Co.

"Alvex (4cc-417)" is a 50% vinyl emulsion of the Calverton Chemical Corp.

The dispersions in the examples in the above formulations are made in substantially the same manner as that shown in Example I. The binder is dissolved in the solvents and the gum adhesive is separately dissolved in water. The water solution is then slowly added to the solvent solution with rapid agitation. In all of the examples given, except Example 6, a slightly alkaline dispersion is more stable. Ammonia or alkali can be used with ammonia being preferred. After coating and drying the coatings become slightly acid. Example 6, Alvex, is acid throughout. The coatings made using the vinyl acetate-maleic anhydride copolymers (having a preponderance of the vinyl acetate) as the continuous phase binder are substantially superior. Another commercial example of this type of resin is Polyco 541 of the American Polymer Corp.

The ratio of water soluble gum to binder can vary be-

tween about 4:1 and 12:1 as shown by the following examples:

| Example No.          | 7   | 8   | 9    |
|----------------------|-----|-----|------|
| $C_3V_{10}$          | 10  | 10  | 10   |
| Toluol               | 60  | 60  | 60   |
| Acetone              | 10  | 10  | 10   |
| Isopropanol          | 10  | 10  | 10   |
| Santicizer E15       | 4   | 4   | 4    |
| NaOH (10%)           | 3.2 | 3.2 | 3.2  |
| Animal glue          | 15  | 30  | 45   |
| Dextrin              | 25  | 50  | 75   |
| Water                | 40  | 80  | 120  |
| Ethyl Acetate        |     | 20  | 25   |
| Ratio, gum to binder | 4:1 | 8:1 | 12:1 |

15 The dispersion technique is critical in making coatings according to this invention. The water-reactivatable adhesive or gum must make up a major portion of the dried film and must be dispersed as a water solution in a solvent solution of a water-insoluble binder. The dispersion must be a dispersion of the water in oil type with the solvent phase as the continuous phase and the water phase as the discontinuous. For this purpose the solvents used to dissolve the binder must be incompletely miscible with water. Solvents can be used for this purpose which are completely 25 water-immiscible, however limited miscibility for the solvent helps to make a stable dispersion. Such limited miscibility can be obtained by using a mixture of solvents, some of which are miscible with water and some of which are immiscible with water. Limited miscibility can also 30 be obtained with a solvent which has a limited miscibility with water by using amounts which are in excess of the amount which would be miscible with the quantity of water used. Sufficient solvent must be used to hold the dispersion to the water in oil type. Thus far at least 35 25% solvent by volume has been required for this purpose. Whether the solvent comprises a single liquid or a mixture of liquids the only requirement is that it be sufficiently immiscible with water to keep the water solution in dispersed phase.

40 The continuous phase binder must adhere to the gum and to the base on which it is coated. The binders of the present invention are substantially water-insoluble which provides increased resistance against washing away of the gumming when moistened liberally and permits lighter coating weights and the use of cheaper and more 45 soluble gums such as dextrans. While the binder is water-insoluble, the water-reactivatable adhesive is readily accessible to remoistening and can be leached almost completely from the dried coating by immersion in water. Apparently the binder structure is quite open and porous.

50 It is believed that this open structure is obtained by the evaporation of water and solvents as the coating is dried. To this end the use of the water-reactivatable adhesive in a water solution rather than as a dry powder is a decided advantage. It has the further advantages of better bonding to the support, permitting the use of higher amounts of water-soluble adhesive, increased speed of activation, lower cost, and because it obviates the need for grinding the gum into very fine particles as taught in the prior art.

60 Some plasticity is desirable in the binder resin and it has been found desirable to add plasticizers to most of the resins used for this purpose. In addition to the plasticizers shown in the examples, plasticizers well known for the particular resins can also be used.

65 To increase quick-tack still further without jeopardizing flatness it is obviously desirable to increase the ratio of glue to resin without making a more nearly continuous glue film or, put another way, to decrease the proportion of resin and yet have enough resin present to keep the glue globules from coalescing completely. Furthermore, flatness could actually be improved if less water were introduced into the system as the glue-resin ratio is increased. As explained above, to avoid the dusting which occurs when dry glue is used in a proportion to resin higher than 70 4:1, a glue solution is emulsified in the resin solution. But

if this glue solution is more than 50% glue it is too viscous to emulsify. Thus, as glue-resin ratio exceeds 6:1 curl begins to increase because it is necessary to add so much water with the glue that the glue globules tend to coalesce too much.

An improvement on the foregoing consists in dissolving water-activatable gum in water to form a water solution of gum, dispersing discrete particles of water-activatable gum in a binder which is incompletely miscible with said water solution and in which said gum is not readily soluble, and dispersing the water solution in said binder to form an emulsion comprising globules of gum in addition to said particles, coating the emulsion on a sheet, and drying the coating while permitting said globules to coalesce partially to form a honeycomb structure of partially coalesced gum particles, the aforesaid binder forming a barrier which prevents said globules from coalescing completely. Before dispersing the water solution in the binder an emulsifying agent should be added to the water solution.

Typical examples for coating paper are as follows, all parts being by weight. In these examples A is the binder solution, B the discrete particles of adhesive, C the water solution and D the emulsifying agent. The carrier and water solutions may also be formulated as in any one of the Examples 1 to 9.

| Examples | 10                                  | 11    | 12    | 13    | 14    |
|----------|-------------------------------------|-------|-------|-------|-------|
| A        | C <sub>3</sub> V <sub>10</sub> 12.5 |       |       |       |       |
|          | Santicizer 141 4.5                  |       |       |       |       |
|          | Toluol 60.0                         | 108.5 | 108.5 | 55.0  | 33.0  |
|          | Ethyl Acetate 22.0                  |       |       |       | 108.5 |
| B        | Isopropanol 9.5                     |       |       |       |       |
|          | Toluol                              |       |       |       |       |
|          | Dextrin (Dry)                       | 25.0  | 50.0  | 55.0  | 77.0  |
|          | Dextrin                             | 33.0  |       |       | 75.0  |
| C        | Animal Glue                         | 67.0  | 75.0  | 75.0  | 50.0  |
|          | Water                               | 100.0 | 100.0 | 100.0 | 100.0 |
|          | (NH <sub>4</sub> )OH (Conc.)        | 2.0   | 2.0   | 2.0   | 2.0   |
|          | Water                               | 2.0   | 2.0   | 2.0   | 2.0   |
| D        | Ratio, Adhesive:Binder              | 10:1  | 10:1  | 20:1  | 33:1  |
|          |                                     |       |       |       | 12:1  |

*Preferred formulas*

| Examples | 15                                  | 16     | 17     | 18     |
|----------|-------------------------------------|--------|--------|--------|
| A        | C <sub>3</sub> V <sub>10</sub> 12.5 |        |        |        |
|          | Santicizer 141 4.5                  |        |        |        |
|          | Toluol 60.0                         | 108.5  | 108.5  | 108.5  |
|          | Ethyl Acetate 22.0                  |        |        |        |
| B        | Isopropanol 9.5                     |        |        |        |
|          | Toluol                              | 20.0   | 20.0   | 20.0   |
|          | Ethyl Acetate                       | 20.0   | 20.0   | 20.0   |
|          | Dextrin (Dry)                       | 60.0   | 60.0   | 60.0   |
| C        | Animal Glue (Dry)                   |        |        |        |
|          | Dextrin                             |        | 15.0   | 100.0  |
|          | Animal Glue                         | 100.0  | 85.0   | 100.0  |
|          | Water                               | 125.0  | 125.0  | 125.0  |
| D        | (NH <sub>4</sub> )OH (Conc.)        | 5.0    | 5.0    | 2.0    |
|          | Water                               | 5.0    | 5.0    | 2.0    |
|          | Ratio, Adhesive:Binder              | 12.8:1 | 12.8:1 | 12.8:1 |

The dry particles of gum should be added to the liquid binder before the water solution of glue is dispersed in the binder. If the dry particles were added to the water solution instead of the liquid binder the particles would be dissolved by the water solution. If the water solution is emulsified in the liquid binder before the dry particles are added, the dry particles combine with the globules of liquid adhesive to produce the same result as if all the adhesive has been dissolved in the water solution; the emulsifying agent is not adequate to keep the dry particles away from the emulsified globules.

After the water solution is dispersed in the liquid binder and before the coating is dried, some water is absorbed by the dry particles from the water solution. Thus the dry particles become swollen and when the coating dries they also coalesce partially so that they are well anchored and do not tend to dust off and so that the coating may contain a larger proportion of gum to binder without curling. The elapsed time between the aforesaid dispersion and drying may vary widely depending upon the de-

gree of coalescence desired but it is preferably within two hours.

As indicated in the above tabulations, in Examples 12 and 13 the binder solution contains additional toluol. In 5 the ratio of adhesive to binder, the adhesive comprises both the dry particles and the coalesced particles of gum and the binder comprises the resinous portion of the binder solution which does not evaporate in drying the gumming. In Example 13 the ratio of adhesive to binder is 33 to 1 and good results have been obtained with ratios as high as 10 35 to 1, and of course the higher the ratio the better so long as the gummed paper remains flat and does not block. Moreover the higher the ratio of adhesive to binder the better the adhesive phase is bound together and to the 15 backing sheet.

By causing the gum particles to coalesce partially the resulting product is quite different from the case where all the particles are applied in dry form and remain discrete. The marked difference between the two products 20 can be demonstrated easily by dissolving out the binder with a solvent which does not dissolve the glue. In the case of the discrete-particle gumming the glue precipitates as powder, while in the partially-coalesced gumming the glue remains as a self-supporting honeycomb structure. 25 This difference affords many advantages.

The partially-coalesced product can have a much higher ratio of glue to binder because the glue helps to anchor the coating to the backing. In the discrete-particle product the coating is anchored to the backing solely by the 30 binder and a larger proportion of binder must therefore be used. Glue being less expensive than binder, this affords a substantial saving in cost.

With the same ratio of glue to binder there is better cohesion in the partially-coalesced product than in the discrete-particle product. Whereas particles of glue tend to 35 "dust off" from the discrete-particle product, the partially coalesced product is free from this objection. This is very important in printing gummed labels. Whereas the discrete-particle product cannot be printed on the gummed 40 side, the partially-coalesced product can be printed on either side. Whereas the dusting of the discrete-particle product tends to clog the type of printing presses, the partially-coalesced product involves no such tendency.

There is better adhesion of the gumming to the backing in the partially-coalesced product than in the discrete-particle product, with the same ratio of glue to binder, this being due to the fact that the glue globules contribute 45 to the adhesion of the gumming to the backing in the partially-coalesced product, whereas the discrete particles of dry glue contribute nothing to this adhesion in the other product.

With the same ratio of glue to binder the partially-coalesced product has quicker tack than the discrete-particle product. While this is due partly to the higher 50 ratio of glue to binder it is probably due more to the porosity of the binder resulting from the evaporation of water from the glue globules during the process of manufacture.

The accompanying drawing is intended to indicate the 55 composition of the gumming and not its structure.

It should be understood that this disclosure is for the purpose of illustration only and that this invention includes all equivalents and modifications which fall within the scope of the appended claims.

I claim:

1. The method of making a substantially non-curling gummed sheet of the water-remoistenable type which comprises dissolving in a solvent a binder which is substantially insoluble in water, dissolving water-activatable gum in water, dispersing the water solution in the binder solution, coating the resulting composition on the sheet and drying, the ratio of gum to binder being at least 4:1 by weight, and the solvent being sufficiently immiscible with water to keep the water solution in dispersed phase.
2. The method according to claim 1, wherein the binder

solvent comprises at least 25% of the liquid by volume in said composition.

3. The method according to claim 1 further characterized in that said binder is dissolved in a solvent mixture comprising a substantially water-immiscible solvent and a solvent having a limited miscibility with water to facilitate the emulsion.

4. Gummed sheet material of the water-remoistenable type comprising a sheet having on one side thereof a dry film which when moistened with water will adhere to a surface, said film comprising a resinous film-forming binder, and a multiplicity of minute particles of water-soluble gum adhering to each other and to said sheet in a honeycomb structure, said binder being substantially insoluble in water but sufficiently open to permit quick activation of said particles by water.

5. Gummed sheet material according to claim 4 where-  
in the binder is selected from the group consisting of poly-  
vinyl ester copolymers, polyvinyl chloride, butadiene-  
styrene copolymers, and substantially water-insoluble  
polymers of acrylic esters.

6. The method of making a substantially non-curling gummed sheet of the water-remoistenable type which comprises dissolving water-activatable gum in water to form a water solution of gum, dispersing dry particles of water-activated gum in a binder solution which is incompletely miscible with said water solution and in which said gum is not readily soluble, and dispersing the water solution in said binder to form an emulsion comprising globules of gum in addition to said particles, coating the emulsion on a sheet, and drying the coating while permitting said globules to coalesce partially to form a honeycomb structure of partially coalesced gum particles, the aforesaid binder preventing said globules from coalescing completely.

7. The method of making a substantially non-curling gummed sheet of the water-remoistenable type which comprises dissolving water-activatable gum in water to

5 form a water solution of gum, dispersing dry particles of water-activatable gum in a binder solution which is incompletely miscible with said water solution and in which said gum is not readily soluble, and dispersing the water solution in said binder to form an emulsion comprising globules of gum in addition to said particles, coating the emulsion on a sheet, and drying the coating while permitting said globules to coalesce partially to form a honeycomb structure of partially coalesced gum particles, the aforesaid binder preventing said globules from coalescing completely and, after said water solution is dispersed in binder and before said coating is dried, absorbing water into said particles from said solution so that they also coalesce partially.

8. Gummed sheet material of the water-remoistenable type which comprises a sheet having on one side thereof a coating of water-activatable gum particles partially coalesced in the form of a honeycomb structure, said particles being withheld from complete coalescence by a binder which is substantially insoluble in water, the ratio of gum to binder being at least approximately 10:1.

9. Gummed sheet material of the water-remoistenable type which comprises a sheet having on one side thereof a coating of water-activatable gum particles partially coalesced in the form of a honeycomb structure, said particles being interconnected by a binder which is substantially insoluble in water, the ratio of gum to binder being at least approximately 10:1.

10. Gummed sheet material according to claim 9 where-  
in the ratio of gum to binder is of the order of 30:1.

#### References Cited in the file of this patent

#### UNITED STATES PATENTS

|    |           |      |       |       |         |
|----|-----------|------|-------|-------|---------|
| 35 | 2,793,966 | 5/57 | Davis | ----- | 117—122 |
|    | 3,104,179 | 9/63 | Prior | ----- | 117—122 |

RICHARD D. NEVIUS, Primary Examiner.